

1

2,790,772

## CUTTING OIL COMPOSITION

Everett C. Hughes, Shaker Heights, and Harrison M. Stine, Lyndhurst, Ohio, assignors to The Standard Oil Company, Cleveland, Ohio, a corporation of Ohio

No Drawing. Application May 19, 1954,  
Serial No. 430,972

2 Claims. (Cl. 252—45)

The present invention relates to a cutting oil concentrate, cutting oils containing such a concentrate and characterized by a unique combination of superior cutting ability and absence of the formation of disagreeable odors when in use, and to a method of making the concentrate.

Oils containing sulfur or sulfur compounds dissolved therein have been suggested heretofore as cutting oils. Such oils also frequently contain chlorine and a fat such as lard oil. It is believed that the sulfur, to be effective in improving the cutting ability of a cutting oil, must be in an active form, i. e., not bound to a carbon atom, which can react with metal being machined under the condition existing at the point of contact between the tool and the machined metal. Heretofore, the amount of active sulfur which could be incorporated into an oil has been dependent largely upon the solubility of free sulfur in the oil and upon the amount of sulfur which can be chemically combined but not bound to a carbon atom.

A great many suggestions have been made heretofore for increasing the active sulfur content of cutting oils. In some instances, these suggestions have resulted in oils having excellent cutting ability but poor odor characteristics and/or stability. In other instances, they have resulted in oils of acceptable odor but of poor cutting ability. Generally it has been found that some compromise must be made among odor, stability, and cutting ability factors, the cutting ability being improved with an increase in sulfur content at the expense, however, of odor and stability.

The odor characteristics of a cutting oil are not necessarily apparent upon an examination of the oil as produced or supplied to a user. In many instances, odors are developed only when the oil is used in machining operations. This is apparently due to the formation of odoriferous compounds under the conditions prevailing at the cutting tool. If the cutting oil develops an unpleasant or obnoxious odor during use, it makes no difference how good the oil is from the standpoint of cutting ability, i. e., the number of pieces that can be machined with a given tool, the wear on the tool and the surface finish of the metal being machined because machinists will refuse to work with it.

Hydrocarbon polysulfides containing one or more alkyl or aryl radicals have been suggested as being suitable for addition to lubricating oils in order to produce cutting oils. Tests have shown that some of this class of hydrocarbon polysulfides, when added to lubricating oils, form compositions having acceptable cutting abilities. Unfortunately, however, most of these hydrocarbon polysulfides, as such and when diluted or blended with a mineral cutting oil base, have obnoxious odors that immediately disqualify them as cutting oil concentrates. Thus, for example, diamyl tetrasulfide has an exceedingly unpleasant odor that is characteristic of the polysulfide itself rather than of a mercaptan impurity, since it cannot be altered by caustic washing, and diallyl tetrasulfide

2

which, because of its light yellow color, ready miscibility with mineral oil and very high sulfur content appeared very promising, was found to have a nauseating garlic odor. The few polysulfides in this group that do not possess such odors initially, almost without exception develop odors, upon use, that are or soon become so obnoxious as to cause machinists to walk off the job. In some instances the odors developed during use do not seem too unpleasant at first but for some reason 10 become intolerable upon continued use due to a subtle accumulation of odors in high speed, automatic, multi-spindle machines, because of the large volumes of oil they require and the heat, violet agitation and splashing to which the oil is subjected.

Proposals to utilize aryl sulfides in cutting oils relate generally to those aryl sulfides in which a sulfur atom or a chain of sulfur atoms is substituted directly on the aromatic nucleus. Thus, for example, proposals have been made to utilize aryl sulfides, such as phenyl-, tolyl-, 15 xylyl-, naphthyl- and anthracene sulfides in cutting oils without suggesting that there are any material differences among the many aryl sulfides that would make some of them less suitable than others.

It has also been proposed in the art to utilize in cutting oils aryl sulfides in which the sulfur atoms or chains of sulfur atoms are connected to the aromatic nuclei by methene or ethene groups. These proposals are limited, however, to aryl sulfides in which one methyl group and, in one unsupported, purely prophetic proposal, two methyl groups, are substituted on the aromatic nuclei and in which the number of sulfur atoms is limited to two despite generalizations as to "polysulfides." It appears to be generally believed in the art that in this more limited class of aryl sulfides, the monosulfides and disulfides are to be preferred over sulfides containing more than two sulfur atoms and the unsubstituted aryl sulfides are to be preferred over substituted aryl sulfides. This preference is apparently based on conclusions by some investigators that the lengthening of the sulfur chain and the substitution of alkyl groups on the aryl nuclei would both contribute to reducing the oil-solubility of such compounds and to making them solid rather than liquid at ordinary temperatures.

The surprising and unexpected discovery has now been made that it is feasible to prepare alkyl-substituted benzyl polysulfides, a term intended herein to include the various isomeric forms of trimethylbenzyl, methylethylbenzyl, propylbenzyl and isopropylbenzyl polysulfides, as well as mixtures thereof, which contain ten carbon atoms in each alkyl-substituted benzyl group and are characterized by appreciably higher total and active sulfur content and molecular weight than has hitherto been considered possible. These compounds have the empirical formula  $C_{20}H_{26}S_x$  and are characterized by the general formula  $R_1-S_x-R_2$  in which  $R_1$  and  $R_2$  are alkyl-substituted benzyl radicals each having a total of ten carbon atoms and  $x$  is between about 4 and 5.  $R_1$  and  $R_2$  may be the same or different so long as each is a trimethylbenzyl, methylethylbenzyl, propylbenzyl or isopropylbenzyl radical. The compounds are liquid at room temperature, readily soluble in cutting oil bases, substantially odorless, and have low volatility and excellent adherence to cutting surfaces at high temperature, all properties that are highly desirable in cutting oils and cutting oil concentrates.

Generally, the method of the invention comprises reacting one or more alkylbenzyl halides containing ten carbon atoms, and therefore including trimethyl-, methylethyl-, propyl- and isopropylbenzyl halides, with an excess of alkali-metal polysulfide and elemental sulfur at an elevated temperature. The reactants may all be mixed together and reacted in a single step. It is preferred, however, first to react one or more of the alkyl-substituted

benzyl chlorides with alkali-metal tetrasulfide to form alkyl-substituted benzyl polysulfides containing an average of at least about three and preferably about four sulfur atoms per molecule. These polysulfides are highly useful as cutting oil concentrates but are then preferably reacted with elemental sulfur to form alkyl-substituted benzyl polysulfides containing an average of between about four and five, and preferably close to five, sulfur atoms per molecule.

In accordance with one embodiment of the method of the invention, preferred because of the ready availability of the starting material, a catalytic reformate containing a mixture primarily of the various isomers of trimethylbenzene and methylethylbenzene is chloromethylated by any suitable means such as, for example, by reaction with formaldehyde, or a formaldehyde engendering material, and HCl in the form of hydrochloric acid, hydrogen chloride gas, or both, for from about two to about seven hours at temperatures of the order of about 150° F. This reaction is advantageously carried out while stirring the reactants under a reflux and, after the reaction is completed to the extent desired, cooling the reaction mixture to room temperature, separating the two immiscible phases, washing the upper oily layer with water and separating the aqueous phase, washing the upper layer with sodium carbonate solution until the products are neutral, separating the layers, washing the products again with water and separating the layers, and finally drying the products with anhydrous calcium chloride. The organic reaction product so obtained after removal of any xylylene dichlorides formed, is a mixture, which may if desired be diluted with unreacted benzenes, of aromatic monochlorides. These monochlorides are primarily the isomers of trimethylbenzyl chlorides having the formula  $(CH_3)_3C_6H_2CH_2Cl$ . Methylethylbenzyl chlorides having the formula  $CH_3(C_2H_5)C_6H_3CH_2Cl$ , and propyl- and isopropylbenzyl chlorides having the formula  $(C_3H_7)C_6H_4CH_2Cl$ , may also be included.

The mixture of aromatic monochlorides obtained in this manner, or any one or combination of alkyl-substituted benzyl chlorides containing ten carbon atoms from any other source, is reacted at an elevated temperature of the order of about 200° F., for several hours with an excess of sodium tetrasulfide in the form of an aqueous solution, preferably with agitation under an inert atmosphere such as nitrogen. Upon cooling and settling, the reaction mixture forms an upper organic phase and a lower aqueous phase. The lower aqueous phase is separated and the remainder, i. e., the upper organic phase, is washed with an alkali-metal hydroxide solution. Upon separation of the alkali-metal hydroxide solution, high yields of alkyl-substituted benzyl polysulfides having ten carbon atoms in each benzyl radical and containing an average of at least about three and generally about four sulfur atoms per molecule are obtained. For convenience, these are referred to herein as alkylbenzyl tetrasulfides.

The reaction between the halides and alkali-metal tetrasulfide is preferably carried out in the presence of a diluent having a low viscosity and a high flash point. Hydrocarbon fractions having boiling points ranging from the kerosene to the fuel oil boiling ranges, generally designated as gas oil, are particularly suitable for this purpose. The addition of a gas oil or fuel oil, which does not react with either the reactants, the alkyl-substituted benzyl tetrasulfides or the ultimately desired alkyl-substituted benzyl pentasulfides, has the highly desirable and purely physical functions of imparting to the mixtures thereof lower viscosities than either the tetrasulfides or the pentasulfides per se, facilitating the handling of the reactants and the products, and aiding in the separation of any aqueous phase after the reaction. Alkyl-substituted benzenes having boiling points above about 300° F., such as any that may be unreacted in the chloromethylation described, are also eminently suitable as diluents. The

diluent remains with the organic phase and serves as such is the succeeding reaction step with elemental sulfur.

The alkylbenzyl tetrasulfides obtained by reaction between the benzyl chlorides and sodium tetrasulfide are then reacted, preferably while remaining in the presence of the diluent, with an excess, preferably 5%, of elemental sulfur for two to three hours at a temperature between about 200° F. and about 300° F., preferably about 240° F., to form the corresponding alkyl-substituted benzyl polysulfides having ten carbon atoms in each benzyl radical and containing an average of between about four and five and preferably close to five sulfur atoms per molecule. For convenience, these are referred to herein as the alkylbenzyl pentasulfides.

In another embodiment of the method of the invention, which involves a higher consumption of sulfur, the alkylbenzyl pentasulfides are prepared directly by admixing alkylbenzyl chlorides simultaneously with an excess of sodium polysulfide and an excess of elemental sulfur and reacting at a temperature below the boiling point of the lowest boiling component in the reaction mixture, e. g., between about 150° F. and about 250° F. The temperature and time of reaction preferred, to avoid settling out of sulfur from the product upon prolonged standing, are about 200° F. and about 2½ hours.

It is to be understood, of course, that it is within the scope of the invention to prepare any one or a selected combination of the possible isomers of the trimethylbenzyl, methylethylbenzyl, propylbenzyl and isopropylbenzyl polysulfides by appropriate isolation of the corresponding isomer or isomers of the starting material.

Both the alkylbenzyl tetra- and pentasulfides, diluted or not with a suitable hydrocarbon diluent such as gas oil, may be blended to form stable and clear solutions with any mineral cutting oil base, e. g., a hydrocarbon oil, such as an acid-treated oil, having a viscosity between about 75 and 300 SSU at 100° F., and said cutting oil base may itself contain free sulfur dissolved therein. The lower limit of viscosity specified is imposed largely by sulfur solubility. Oils having viscosities higher than 300 SSU at 100° F. are not preferred because of difficulties of handling and flowing. Cutting oil blends containing as little as 0.5% or less by weight of alkylbenzyl tetrasulfide or pentasulfide have excellent cutting ability. Concentrates containing as much as about 50% to 70% or more of alkylbenzyl polysulfide in gas oil or other hydrocarbon diluent, without being blended with a cutting oil base, have superior cutting ability and excellent odor characteristics. The concentrates of the invention, apparently because of their higher molecular weight and surprisingly high content of active sulfur, combine this unusually excellent cutting ability with low volatility, ability to stay on the tool and the work at the cutting point, absence of objectionable odor either upon standing or in severe use and ability to form stable blends with mineral cutting oil bases. For cutting operations on ductile steels, sulfurized oil blends containing between about 0.5% and about 5% by weight of the concentrate are highly satisfactory.

Perhaps the most surprising characteristic of the alkylbenzyl tetrasulfide and pentasulfide cutting oil concentrates of the invention is that they make it possible to incorporate into a cutting oil blend more active sulfur than is required or desired for some types of cutting operations. The present invention, therefore, provides an excellent means of controlling accurately the amount of active sulfur in a cutting oil so that it will be the optimum amount for any particular metal cutting operation. It is also possible to add small amounts of other ingredients, e. g., 1% by volume lard oil, that mask the effect of excess active sulfur.

It is to be understood that while the products of this invention consist essentially of one or a combination of alkyl-substituted benzyl polysulfides containing ten carbon atoms in each benzyl group, preferably diluted with

unsulfurized gas oil or blended with a mineral cutting oil base or both, conventional additives such as lard oil, graphite and oil-soluble chlorinated compounds such as chlorinated wax and chlorinated aromatics typical of which is chlorinated biphenyl and the like may be added in amounts that do not materially alter the character of the products. It is also within the scope of the invention to add minor proportions, i. e., of the order of 1% or less, of antioxidants.

The blending of the cutting oil of the invention with lard oil in an appreciable amount, i. e., above about 1%, and preferably from about 2 to 10% by volume, is particularly desirable and advantageous for reducing tool wear when cutting operations are carried out on abrasive steels and has the further advantage of providing a cutting oil that is most universally useful on both abrasive steels and ductile steels. One example of such a preferred cutting oil is a blend of a mineral cutting oil base with about 4% by volume lard oil and about 1% by weight of a 60/40 mixture of alkylbenzyl polysulfide and gas oil. It is to be understood, therefore, that it is within the scope of the invention to add amounts of lard oil which do alter somewhat the character of the alkylbenzyl polysulfide-containing cutting oils of the invention in so far as the machining of abrasive steels is concerned.

The advantages and utility of the cutting oil concentrate, cutting oil and method of this invention will become more apparent from the following example illustrating the invention.

#### EXAMPLE

##### Part A

120 parts by weight of "Solvesso 100," a catalytic reformate comprising a mixture of 4% aliphatic hydrocarbons and 96% aromatic hydrocarbons containing approximately 39% by weight trimethylbenzene isomers (7% 1,3,5-trimethylbenzene, 27% 1,2,4-trimethylbenzene and 5% 1,2,3-trimethylbenzene), 36% by weight methyl-ethylbenzene isomers (20% 1-methyl-3-ethylbenzene, 8% 1-methyl-4-ethylbenzene and 8% 1-methyl-2-ethylbenzene), 3% isopropylbenzene and minor amounts of m-xylene (3%), o-xylene (6%), p-xylene (trace) and (13%) unidentified monoalkylbenzenes probably including n-propylbenzene isomers, were refluxed at 140 to 158° F. for seven hours under a water condenser while stirring the reactants with 525 parts by weight of 36% aqueous hydrochloric acid and 42.8 parts by weight of 91% paraformaldehyde in the form of flakes. During the reaction a slow stream of HCl gas was fed to the reaction mixture and care was taken to provide good ventilation. After seven hours, the reaction mixture was cooled to room temperature and allowed to settle into two immiscible layers, the lower aqueous layer was separated, the upper oily layer was washed with water, then washed with a 5% aqueous sodium carbonate solution until neutral and then washed again and finally dried with anhydrous calcium chloride.

55% of the final oily phase was found to be a mixture of alkyl-substituted benzyl chlorides having the empirical formula  $C_{10}H_{13}Cl$ , 19% was found to be a mixture of alkyl-substituted xylylene dichlorides and the remaining 26% was found to be substantially unreacted. The products were then subjected to vacuum distillation to separate the alkylbenzyl chlorides and unreacted alkylbenzenes from the alkylxylylene dichlorides.

##### Part B

168.5 parts by weight of the alkylbenzyl chlorides of Part A were admixed with 368 parts by weight of a 40% aqueous solution of sodium tetrasulfide (approximately a 30% excess of the tetrasulfide to insure complete reaction of the chloride) and with 132 parts by weight of a gas oil having a viscosity of 42 SSU at 100° F. and a flash point at 275° F. The mixture was heated to 200° F. and maintained at that temperature for from 3 to 5

hours while stirring well. The reaction products were then cooled and allowed to settle, the lower aqueous phase was separated and the remaining organic phase was hydroxide solution per 5 parts by volume of organic phase, and the mixture was stirred for thirty minutes, the caustic then being separated. Thereupon, 3% Super Filtrol, a mineral adsorbent, was added and the mixture stirred for about ten minutes. The mixture was then filtered to yield 94 to 99% of the theoretical yield of alkylbenzyl polysulfides in the gas oil.

The product was a 60/40 mixture of alkyl-substituted benzyl tetrasulfides, having the empirical formula  $C_{20}H_{26}S_4$ , and gas oil having a total sulfur content of 18.5% (95% of the theoretical 19.4% total sulfur content, or containing an average of about four sulfur atoms per molecule of polysulfide) and an active sulfur content of 8.7% (90% of the 9.7% theoretical active sulfur content).

##### Part C

329 parts by weight of the 60/40 mixture of alkylbenzyl tetrasulfide and gas oil prepared in accordance with part B of the example were admixed with 16 parts by weight of elemental sulfur and sufficient additional gas oil, about 10 parts by weight, to maintain the ratio of polysulfide to gas oil at about 60/40. The mixture was then stirred for 2 hours under nitrogen atmosphere at a temperature of 240° F.

The total sulfur content of the alkyl-substituted benzyl pentasulfides, likewise having the empirical formula  $C_{20}H_{26}S_5$ , analyzed 22.9% (98% of the theoretical 23.5%, or containing an average of about five sulfur atoms per molecule) and the active sulfur content analyzed 15.1% (105% of the theoretical active sulfur content of 14.3%). The amount of sulfur introduced was about equal to the theoretical amount considering the precision of the available analytical methods.

##### Part D

40 A cutting oil base was prepared by adding, to Diamond Paraffin oil, an acid treated lubricating oil stock having a viscosity of 100 SSU at 100° F., 0.8% by weight elemental sulfur, i. e., the maximum amount of sulfur soluble in the oil at 0° C. The mixture was heated and stirred at 240° F. until all of the sulfur was dissolved. This took approximately one to two hours.

Blends of the cutting oil base with 0.5 to 5% by weight of the 60/40 alkylbenzyl tetrasulfides-gas oil concentrate prepared in Part B of the example and with 0.5 to 5% by weight of the 60/40 alkylbenzyl pentasulfides-gas oil concentrate prepared in Part C of the example form excellent cutting oils characterized by remarkable cutting ability, low volatility and absence of odor, and ability to remain on the work and the tool at the point of cut.

55 A blend of cutting oil base with 1% by volume of the 60/40 alkylbenzyl pentasulfide-gas oil concentrate, 4% lard oil and 0.5% "Aroclor 1254," a chlorinated biphenyl available as a yellow-tinted, viscous oil having a chlorine content of 54%, a specific gravity between 1.538 and 1.548 and a distillation range of 365-390° C., was found to be particularly effective.

It is obvious that in the foregoing example bromine or iodine can be substituted for chlorine and that likewise potassium tetrasulfide can be used in place of sodium tetrasulfide. Chlorine, alkyl-substituted benzyl chlorides, and sodium tetrasulfide are preferred because they are relatively inexpensive and most readily available.

It is to be understood that these and other modifications of the method and products described herein will readily occur to those skilled in the art. All such modifications are intended to be included within the scope of the invention as defined in the accompanying claims.

We claim:

1. A cutting oil concentrate comprising from about 50 to about 70% by weight of a mixture of organic poly-

treated with one part by volume of a 3% aqueous sodium sulfides having the formula



wherein R<sub>1</sub> and R<sub>2</sub> are selected from the group consisting of three methyl radicals, one methyl and one ethyl radical, and one propyl radical, and x averages between about 4 and 5, said mixture having been derived from a mixture of aromatic hydrocarbons containing approximately 9% xylenes, 3% isopropyl benzene, 36% methyl ethylbenzenes, 39% trimethylbenzenes, and 13% mixed monoalkylbenzenes, by chloromethylation and reaction with sodium tetrasulfide, and with sulfur when x is in excess of 4, and from about 50 to about 30% by weight of a hydrocarbon diluent.

2. A cutting oil comprising a mineral oil and from about 0.5 to about 5% by weight of a mixture of organic polysulfides having the formula



where R<sub>1</sub> and R<sub>2</sub> are selected from the group consisting of three methyl radicals, one methyl and one ethyl radical, and one propyl radical, and x averages between about 4 and 5, said mixture having been derived from a mixture of aromatic hydrocarbons containing approximately 9% xylenes, 3% isopropyl benzene, 36% methyl ethylbenzenes, 39% trimethylbenzenes, and 13% mixed monoalkylbenzenes, by chloromethylation and reaction with sodium tetrasulfide, and with sulfur when x is in excess of 4.

#### References Cited in the file of this patent

##### UNITED STATES PATENTS

|           |                    |               |
|-----------|--------------------|---------------|
| 2,113,092 | Moran et al. ----- | Apr. 5, 1938  |
| 2,185,008 | Wojcik -----       | Dec. 26, 1939 |
| 2,273,471 | Kimball -----      | Feb. 17, 1942 |
| 2,538,941 | McCallum -----     | Jan. 23, 1951 |
| 2,676,987 | Lewis et al. ----- | Apr. 27, 1954 |